

A. M. CRAIG.

## ART OF CASTING METALS.

APPLICATION FILED DEC. 6, 1913.

1,107,905.

Patented Aug. 18, 1914



Digit:



314



Fig: 2



3.

Witnesses:

Stein Mc. Craig, Inventor  
By his Attorney,  
W. D. Hutchinson,

# UNITED STATES PATENT OFFICE.

ALVIN M. CRAIG, OF NEW HAVEN, CONNECTICUT.

## ART OF CASTING METALS.

1,107,905.

Specification of Letters Patent. Patented Aug. 18, 1914.

Application filed December 8, 1913. Serial No. 805,225.

To all whom it may concern:

Be it known that I, ALVIN M. CRAIG, a citizen of the United States, residing at New Haven, county of New Haven, and State of Connecticut, have invented a new and useful Improvement in the Art of Casting Metals, of which the following is a full, clear, and exact description.

My invention relates to improvements in the art of casting metals, and the object of my invention is to produce a method or improvement in the art whereby metals can be rapidly cast, the metal of the casting compressed during the operation so that an exceedingly dense casting will be produced, to provide means of leaving the surface of the casting smooth, to utilize metal molds for this purpose, to compress the metal so that the reaction caused by the swell of the poured metal and the expansion of the mold, can be taken up without injury to either casting or mold, and use air pressure in such a way that the exhaust from the air pressure device can be utilized to chill the mold and cool the casting.

Where metals are cast in a solid mold and then submitted to pressure as in the plunger type of compression casting apparatus, there is great liability of cracking the mold or casting, or of distorting the latter; and this is especially so where hydraulic or inelastic means of compression is used, and where spring sections are used in the molds the pressure is insufficient, and the heated mold quickly destroys the temper of the springs. In carrying out my invention, however, I use a two-part mold which is expandible both laterally and longitudinally, and which consequently when pressure is applied to the mold, permits of compression in all directions. I use an air engine for effecting the compression so that the reaction caused by the swelling of the poured metal or mold will act against the air, and I can utilize the engine exhaust for cooling the mold and metal. This will be best understood by the description which follows.

Reference is to be had to the accompanying drawings forming a part of this specification, in which similar reference characters indicate corresponding parts in all the views.

Figure 1 is a broken side elevation of a simple form of apparatus capable of carrying my process into operation. Fig. 2 is an enlarged cross section of a closed mold.

Fig. 3 is a perspective view of the two-part mold with the parts slightly separated, and Fig. 4 is a detail view showing the pivotal connection between the piston rod and one of the mold sections.

I have shown a very simple means of carrying the invention into effect, and it will be understood that very many other forms of apparatus can be used for accomplishing the same result. As illustrated the apparatus has a suitable base frame 10 formed of spaced apart side rails, and at the end of the frame are brackets or abutments 11 to one of which is fixed a mold section 12 comprising half the mold, while the opposed section 13 reciprocates with relation to the section 12. Each of these sections is provided with side walls or wings 14 and 15, placed at right angles to each other, the edge of the wall 15 abutting with the opposed wall 14 of the other section, when the mold is closed as shown in Fig. 2, and the walls 14 are preferably provided with raised portions or shoulders 14<sup>a</sup> which set into the mold so as to make a close joint.

At the top the section 12 has a cover 16 closing over the top of the opposed section 13 when the parts of the mold are put together, and the member 13 has a bottom section 17 which closes over the bottom of the section 12 so that when the sections are pushed together, the metal can be poured and the mold sections are held under pressure so that the metal is greatly condensed, while the swelling action of the casting or metal, if excessive, will cause the sections of the mold to yield against their elastic backing sufficiently to prevent breaking of the mold or casting, or distortion of the latter.

The mold is provided with a suitable ingate 18 at the top. As a means of guiding the reciprocating mold section 13, it has trucks 19 on the side running on supporting rails 20. At the back of the section 13 it has a loose connection as shown at 21 with a piston rod 22 connecting with the piston of the cylinder 23 which is suitably supported and backed by one of the abutments or brackets 11. The above connection can be made by simply passing a pin 21<sup>b</sup> through the casing 21<sup>a</sup> on the back 14 of the mold section and through the piston rod 22 which enters said casing, although any suitable loose connection between the piston rod and mold can be used. The air is admitted un-

der pressure through a three-way cock 24 having connections at 25 and 26 with the ends of the cylinder 23, and the exhaust also comes back through the pipe 26 and connects 5 with a pipe 27 leading to the cross-pipe 28, and this has jet openings 29 discharging upon the sections 12 and 13 when the mold is open. I have not shown the details of the pipe connection with the cylinder 23, or the 10 arrangement of the piston, because this arrangement is common to many forms of apparatus, and I use any preferred type of air engine and pipe connection.

When the apparatus is used, the cock 24 is 15 turned so as to actuate the engine, and the piston throws out the rod 22 and slides the section 13 against the section 12 so as to close the mold. The metal is then poured, and air is then admitted to the cylinder or engine 20 23 so as to greatly compress and condense the metal in the mold. When the metal is first poured and before it begins to cool, it swells quickly, and the mold sections also 25 swell under the heat; but as the pressure back of the piston is an elastic one, the mold can react against this pressure, and this yielding of the mold will prevent injury to either the mold or the casting. Additional pressure can then be admitted to the cylinder 30 23 so that the metal while soft can be compressed to any desired extent. The piston in the cylinder 23 is then reversed, thus opening the mold, and the casting can drop from the mold, being started manually or 35 otherwise if necessary. As the mold is opened, the exhaust from the cylinder 23 passes through the pipes 27 and 28, and the expanding air is directed against the mold sections 12 and 13, and the casting in the 40 latter, so that the said parts are quickly chilled. This will be readily understood because it is well known that when air is allowed to expand quickly after being heavily compressed, it absorbs the surrounding heat 45 to such an extent that the adjacent parts become exceedingly cold.

It will be seen that by means of this process I can get a very dense smooth fine casting, and it will be noticed that the air blast 50 will keep the mold cool to a certain extent so that casting can be carried on continuously and with great rapidity. I thus get the double advantage of great speed in casting, and a much better casting than can be produced in ordinary ways. It will be seen 55 that this arrangement is adapted for rapid casting, especially as the mold can be so readily opened and closed, and as provision

is made for preventing the mold from being unduly heated. It will also be observed that 60 in my improved process I use a two-part mold which practically forms a container or bottle in which the liquid is poured, and that I am able to apply a heavy but elastic pressure to the mold in all directions so as to 65 hold the liquid metal against expansion, and thus greatly condense it, and that I use air as the compression means so that in case of 70 extraordinary expansion for any reason, the compression force is in the nature of a cushion which will permit slight reaction of the mold against the air cushion without danger of breaking the mold. It will also be seen that I can apply the pressure instantly because the mold parts are held firm, and the 75 liquid metal begins to be condensed as it cools. This is quite different from the process in which plungers are used to squeeze the metal in two directions, and in which the metal is permitted to first chill on the outside 80 before the compression force is applied.

I claim:—

1. The herein described method of casting metals which consists in pouring the metal into a mold which is laterally and longitudinally expansible and applying a heavy but elastic pressure to the mold and metal while the metal is still liquid and before it has had time to set. 85

2. The herein described method of casting 90 metals, which consists in bringing the mold parts together, pouring the metal into the mold, and holding the mold parts together by a heavy but elastic pressure acting on all parts of the mold, thereby condensing the 95 molten metal as soon as it is poured.

3. The herein described method of casting metals, which consists in pouring the melted metal into a compressible and expansible mold, forcing the mold sections upon the 100 metal by an air pressure, and cooling the mold sections when the mold is opened by a blast of compressed air. 105

4. The herein described method of casting metals, which consists in pouring the melted metal in a compressible and expansible mold, maintaining the metal in the mold in compressed condition by air in an air engine, and directing the exhaust of the engine upon the mold sections when the mold is opened 110 for the purpose of cooling said mold sections.

ALVIN M. CRAIG.

Witnesses:

WARREN B. HUTCHINSON,  
ARTHUR G. DANNELL.